

## UNITED STATES PATENT OFFICE.

WALTHER MATHESIUS, OF CHARLOTTENBURG, GERMANY.

## ALLOY OF LEAD AND ALKALINE EARTH METAL.

No Drawing.

Application filed May 16, 1921. Serial No. 469,959.

*To all whom it may concern:*

Be it known that I, WALTHER MATHESIUS, a citizen of the German Republic, residing at Charlottenburg, Germany, have invented 5 certain new and useful Improvements in an Alloy of Lead and Alkaline Earth Metal, for which I have filed application for patent in Germany on January 7, 1920, of which the following is a specification.

10 This invention relates to an alloy of lead with metals of the alkaline earths, calcium, strontium, barium. An alloy of lead with about 3% of calcium, and containing also about 1-3% of cadmium or bismuth or both, 15 has been described in the German Patent No. 297210.

Metallographic examination of the alloy in question shows that substantially harder 20 crystals are embedded in uniform distribution in a homogeneous main mass. On closer examination of the texture, it can be easily shown that these harder crystals are constituted by an alloy of lead and calcium, the composition of which may be considered 25 as corresponding to the formula  $Pb_2Ca$ . This lead-calcium compound is soluble in molten lead and during the process of solidification of the main body of lead, crystallizes out of the latter so that this process 30 produces a uniform distribution of the calcium-lead in the whole of the rest of the alloy.

In the above mentioned alloy of the German Patent 297210, the addition of the 35 metals cadmium and bismuth is intended to harden the main lead portion of the alloy to a certain extent and to reduce its melting point, moreover, as owing to the addition even of a few per cent of calcium to 40 lead, the melting point of the latter is considerably raised.

A metal of the composition referred to is 45 eminently suitable, as shown by experience, for use as metal for lining bearings in the same manner in which the so-called "tin-white metals" have been exclusively employed. As shown by metallographic examination, even in good tin-white metals, the structural conditions are exactly the 50 same, only here the harder crystals are uniformly distributed in the softer main mass, are composed of a copper-tin alloy.

In both cases the harder crystals embedded 55 in the softer main mass, form, during the use of the alloys as bearing metals, those ingredients of the alloy which, after a cer-

tain running-in of the shaft has taken place, form the bearing surface proper.

Exhaustive experiments have now proved 60 that it is possible to obtain alloys which are eminently suitable for use as bearing metals, exclusively from lead with an addition of calcium, strontium, and barium, and without cadmium or bismuth.

The metals, strontium and barium, form 65 with lead definite chemical compounds exactly in the same way as calcium. Metallographic examination of the texture of such an alloy on a ground surface shows that strontium-lead alloy is exactly similar to 70 calcium-lead alloy in a peritectic structure, whilst barium-lead compound solidifies with the excess of lead at the same time to form a eutectic.

The barium-lead compound produces 75 therefore in the alloy chiefly a hardening of the main mass, whilst strontium-lead like calcium-lead, chiefly assists in the formation of harder crystals.

Examination of melting or softening temperatures of such alloys shows, however, 80 that when the alloy solidifies, the three compounds do not completely crystallize out of the same, on the contrary some traces of the said compounds are still left in the alloy in 85 the state of solid solution, for a considerable lowering of the melting or softening temperature takes place when, in addition to calcium which is most easily obtained in large quantities, are also added to the alloy 90 certain quantities of strontium or barium, or preferably, both.

While the addition of the calcium to the lead increases the melting temperature, the addition of two, (or still better, all three) 95 of the alkaline earth metal ingredients, produces a lowering of the melting temperature and increases the fluidity of the alloy with in moderate limits.

On these observations is based the manufacture of a new bearing metal alloy from lead with about 3% calcium or about 1% each of strontium and barium.

It is possible to produce an alloy of such 100 composition having a degree of hardness of 35-40 Brinell units, the said alloy having a melting point of 450-500° C. and therefore being excellently adapted for use as bearing metal.

Metallographic tests have shown that, in 110 an alloy of this kind, an extremely uniform distribution of the harder crystals exists,

which has heretofore only been true of the best tin-white metals. In itself, the proposition, to add alkaline-earth metals to the lead, is not new. But at the most, only two alkaline-earth metals have heretofore been added to the lead, or if three such metals have been used, it has been considered necessary to further add other metals to affect the physical properties of the alloy. It has never before been realized that, by the addition of calcium to the lead, there can be obtained the formation of the hard lead-calcium crystals and that, by the addition of barium and strontium, there results a hardening of the basic mass, and, at the same time, a lowering of the melting point, which is increased considerably by the addition of the calcium. This commercial result which as stated, is reproduced in the metallographic image, can only be obtained when the proportions stated for the additions of the three alkaline-earth metals, (viz., about 3% calcium and about 1% each of strontium and barium), are maintained. The applicant has proven by tests that only with these

proportions can an alloy be produced having the desired hardness of the basic mass and the uniform distribution of the crystals, together with a satisfactory liquidity.

I claim:

1. A lead alloy containing about 3% of calcium and about 1 to 2% of another alkaline earth metal, such alloy being substantially free from metals other than those stated.

2. An alloy of lead containing about 3% of calcium and about 1% each of strontium and barium, such alloy being substantially free from metals other than those stated.

3. An alloy of lead containing about 3% of calcium, together with smaller percentages of strontium and barium, such alloy being substantially free from metals other than those stated.

In testimony whereof I affix my signature in presence of two witnesses.

WALTHER MATHESIUS.

Witnesses:

OTTO SCHNEIDER,  
GERTRUD DOMKONSKI.